

Aug. 26, 1958

L. B. PALMER

2,849,335

BACKING FOR SMOOTH SURFACE COVERINGS AND PROCESS THEREFOR

Filed Sept. 17, 1956



FIG. 1



FIG. 2

INVENTOR.  
LEON B. PALMER

BY *William T. Wies*

AGENT

1

2,849,335

BACKING FOR SMOOTH SURFACE COVERINGS  
AND PROCESS THEREFOR

Leon B. Palmer, Little Falls, N. J., assignor to Con-goleum-Nairn Inc., Kearny, N. J., a corporation of New York

Application September 17, 1956, Serial No. 610,238

33 Claims. (Cl. 117—68)

This invention relates to smooth surface coverings for floors, walls, and the like. In particular, it relates to fibrous sheets suitable as backings for such coverings and to methods of producing them.

Smooth surface coverings such as linoleum, printed felt base and the like are made up of a decorative layer applied to a sheet of fibrous backing material. The decorative layer may have wear-resistant properties or a transparent wear-resistant coating may be applied thereto. The product is then adhesively bonded to the surface to be covered. According to conventional practice, the fibrous back is uniformly impregnated throughout with a binder, such as a bituminous material, thereby providing a satisfactory backing sheet for the product from the standpoint of strength, water resistance, and resistance to indentation.

A product comprising such a uniformly impregnated backing is characterized, however, by requiring an excessively long time for setting the adhesive when it is installed. The decorative and wear-resistant layer tends to develop cracks caused by lateral shifting of the base to which the product is bonded. Such shifting is commonly due to varying conditions of humidity in the surrounding atmosphere. Furthermore, if replacement is desired, removal of the product is difficult due to the inherent strength of the backing in resisting delamination.

Consequently, it has been proposed that a nonuniformly impregnated backing be used. Such a backing comprises a sized zone having a relatively small amount of binder and an impregnated zone having a greater amount of binder. A backing sheet of this type is disclosed in U. S. Patent 2,295,070.

In the production of a surface covering comprising such a backing, the decorative layer is applied to the side of the backing bearing the impregnated zone. During installation, the side bearing the sized zone is adhesively bonded to the surface to be covered. A product of this type is characterized by rapid setup of the adhesive when it is bonded to a surface, ability to withstand lateral shifting of the surface upon which it is installed without cracking of the wear layer, and ease of removal from the surface if replacement is desired.

There is, unfortunately, a disadvantage which tends to offset these advantages. The fibers in the sized zone of the backing sheet tend to swell while the adhesive is becoming set. This leads to growth of the whole backing sheet, causing the edges of the sheet to curl upwards, a phenomenon called "tenting." Tenting of the seams in a surface covering installation is objectionable since the location and presence of the seams is emphasized and also since the seams are then areas of potential weakness in the installation.

The cure for tenting which has been used in the past has been to increase the thickness of paint applied to the side of the backing sheet which is bonded to the surface to be covered. This heavy backing paint, however, has drawbacks, including increased material cost, increased tendency of the painted back to develop cracks,

thus detracting from the salability of the product, greatly increased setup time for the adhesive, and poorer adhesion of the adhesive due to the slicker, smoother back surface of the product.

It is an object of the invention to provide a surface covering comprising a fibrous backing and a decorative layer characterized by the ability to be quickly and firmly bonded to a surface without objectionable tenting of seams. It is a further object of the invention to provide a surface covering with a fibrous backing which can be quickly and firmly bonded to a surface without tenting of the seams characterized by ease of removal for replacement purposes. Other objects and the advantages of the invention will appear hereinafter.

In accordance with the invention, a fibrous sheet is sized from one side with a sizing solution comprising a binder and a small amount of an organopolysiloxane. The sheet is impregnated from the other side with a greater amount of binder so that no dry felt remains within the sheet to produce a product which comprises a sized zone and an impregnated zone. The sized and impregnated sheet is a suitable backing for a decorative surface covering product.

With reference to the drawing,

Fig. 1 is a cross-sectional view of a fibrous sheet impregnated according to the invention;

Fig. 2 is a cross-sectional view of a surface covering installation formed by laminating a wear layer to the sheet of Fig. 1 and bonding the product to a surface.

A fibrous sheet 1 is impregnated and sized with binder so as to create an impregnated zone 2 with greater binder content and a sized zone 3 of lesser binder content. The zone 3 contains a small amount of an organopolysiloxane. An overlap zone 4 comprising binders used in both the impregnated and sized zones and organopolysiloxane is between the sized and impregnated zones within the sheet. A seal coat 5 is applied to the surface of the zone 2 and a coat 6 of backing paint is applied to the surface of the zone 3. A layer 7 of decorative wear-resistant composition is laminated to the seal coat. The product is bonded to a surface 8 by means of an adhesive layer 9.

The fibrous sheet is preferably a web of felted fibers. The felt is generally produced using a Fourdrinier or cylinder paper machine with the thickness of the resulting sheet normally falling in the range of from 0.02 to 0.08 inch. The fibrous material used for making the felt is normally cellulose in origin although other fibers can be used including those of mineral and animal origin. The sources of cellulose material can include cotton or other rag stock, wood pulp, including both ground wood and chemical wood pulp, paper, boxes, or mixtures thereof in any proportion. The sheet can also contain fillers such as wood flour.

The density of the fibrous sheet useful as a backing for a surface covering is lower than that of paper. The physical characteristics of a sheet of this type are commonly defined by the ratio of the thickness of the sheet to the weight of a specified area. This ratio is often referred to as the gauge to weight ratio. It is preferred that the fibrous sheet used as a backing according to the invention have a gauge to weight ratio in excess of 0.8 as defined by the formula:

$$\frac{\text{Thickness of felt (thousandths of an inch)}}{\text{Weight of 480 sq. ft. of dry sheet (pounds)}}$$

A particularly effective range of gauge to weight ratios is from 0.8 to 1.2. These values are to be contrasted with the gauge to weight ratio of paper which is normally about 0.4 and rarely exceeds 0.8.

In accordance with the invention, one side of the fibrous sheet is sized to a controlled depth with a dispersion of

sizing binder in the presence of a small amount of a soluble organopolysiloxane. The binder used in the sizing solution is any of the well-known binders which are commonly used for imparting strength and water resistance to a fibrous sheet. Such resinous binders as urea-formaldehyde and phenol-formaldehyde resins, polyvinyl chloride, polyvinyl acetate, vinyl chloride-vinyl acetate copolymer, butadiene-acrylonitrile copolymer, butadiene-styrene copolymer, polymers and copolymers of acrylic acid and the like can be used. The preferred binder, for reasons of low cost and the desirable properties which it imparts to the fibrous sheet, is a bituminous material and is usually an asphalt of either petroleum or natural origin or blends of the two. The preferred bituminous binder can be crude, blown or steam distilled and can, in addition to asphalts, be tar or pitch residues of vegetable and animal origin. Normally, the bituminous binder used in the sizing solution has a softening point of between about 130° F. and about 200° F.; preferably, the softening point is between 170° F. and 190° F.

The organopolysiloxanes effective in the invention are characterized by having a plurality of silicon atoms linked together through oxygen atoms with at least one hydrocarbon radical attached to each silicon atom. Such hydrocarbon radicals include alkyl, such as methyl, ethyl, propyl, isobutyl, isoamyl, amyl, hexyl, heptyl, octyl and the like; aryl, such as phenyl and the like; alkaryl, such as tolyl, xylol and the like; aralkyl, such as benzyl, phenylethyl and the like; and cycloalkyl, such as cyclopentyl, cyclohexyl and the like. The repeating structure in the molecule is:



where  $\text{R}_1$  is a hydrocarbon radical having from 1 to 8 carbon atoms and  $\text{R}_2$  is either a hydrocarbon radical having from 1 to 8 carbon atoms or hydrogen.

Organopolysiloxanes wherein at least one of the radicals attached to each silicon atom is a methyl group are particularly effective in the invention. These preferred polymers include dimethyl polysiloxane, methyl phenyl polysiloxane, methyl hydrogen polysiloxane, methyl ethyl polysiloxane and the like.

The organopolysiloxanes effective in the invention are prepared by any of the well-known methods of preparation of such materials. For example, the hydrolysis of a disubstituted silicon dichloride produces a disubstituted silicon compound with two  $-\text{OH}$  groups. Two or more of these molecules can join, splitting out water to form the siloxane bonding.



and so on.

The condensation of molecules containing Si bonded to  $-\text{OH}$  groups can continue to any degree to produce products of varying viscosity. The polymerization can be influenced by catalysts such as sulfuric acid, sodium hydroxide, copper hydroxide, fennic sulfate, sodium sulfate and the like. The products can be linear polymers or cross-linking can take place during the polymerization.

To be effective in the invention, the organopolysiloxanes should either themselves or their concentrated solutions be of sufficient fluidity so that they be readily dispersed in the sizing solution, and so that their presence does not impart to the sizing solution so high a viscosity

that absorption of the solution by the fibrous sheet becomes difficult. It is preferred that the viscosity at 77° F. of a dispersion comprising 90 percent organopolysiloxane and 10 percent xylene be from about 5 to about 5000 centistokes. A particularly effective range of viscosities at 77° F. of the dispersion is from 10 to 100 centistokes.

The organopolysiloxanes effective according to the invention should be very low in free acidity, as any appreciable free acid tends to promote the formation of sludge in the sizing solution. It is preferred that the acid number of the organopolysiloxane (defined as the number of milligrams of potassium hydroxide required to neutralize 1 gram of polymer) be less than 0.4. In addition, the solvents used to prepare the sizing solution should be dry since organopolysiloxanes tend to react with water with the formation of a flocculent precipitate.

The effective organopolysiloxanes are further characterized by being heat hardenable; that is, they are adapted to be cured by heat to a tough solid form. The cure of these effective organopolysiloxanes can proceed at varying rates at ordinary temperatures, but the application of heat accelerates the curing process. In the curing process, cross-linking and polymerization takes place within the organopolysiloxane molecule.

In producing the polysiloxane containing sizing solution for use in the invention, a dispersion of binder in solvent is first prepared. Such solvents as kerosene, naphtha, methyl ethyl ketone, methyl isobutyl ketone, carbon tetrachloride, toluene, xylene, turpentine, diethyl ether, perchloroethylene, Stoddard solvent and the like can be used. The binder can be in solution in the solvent or as an emulsion in the presence of conventional emulsifying agents.

Organopolysiloxane, preferably also dispersed in a solvent that is miscible with the solvent used for dispersing the binder, is added to the dispersing of binder. A common solvent for dispersing the organopolysiloxane is xylene, but other solvents such as those listed above can be used.

The sizing solution normally contains about 0.2 to about 10 percent organopolysiloxane and about 10 to about 50 percent sizing binder with the balance being made up of solvent. The presence of organopolysiloxane in higher concentrations than 10 percent results in an unstable dispersion of the sizing solution from which impregnant has a tendency to be displaced from solution. A particularly effective range of composition for the sizing solution is 0.5 to 1.25 percent organopolysiloxane, 20 to 40 percent sizing binder and the balance solvent.

The depth of penetration of the fibrous sheet by the sizing solution is controlled by varying the time of contact of the sheet with the solution and by the pressure exerted by the squeeze rolls between which the sheet passes for the purpose of removing surplus sizing solution. The depth of sizing is normally from about 20 percent to about 70 percent of the thickness of the sheet. A particularly effective range is from 30 percent to 60 percent of the thickness of the sheet.

The fibrous sheet, after being dried for removal of the solvents used for dispersing the impregnant, is then impregnated from the side opposite to that which has been sized. The impregnating binder can be any of the resinous binders disclosed as useful as sizing binders. For reasons of cost and the desirable properties which it imparts to a fibrous sheet, a bituminous impregnating binder is preferred.

The preferred binder is conventionally an asphalt of either petroleum or natural origin or blends of the two. The bituminous binder can be crude, blown or steam distilled and, in addition to asphalts, can be tar or pitch residues of vegetable and animal origin. Normally the bituminous impregnating binder has a softening point of between about 100° F. and about 160° F.; preferably, the softening point is between 140° F. and 150° F.

The impregnation step in the case of use of the preferred bituminous binders is normally carried out by hot

melt application; that is, a molten bath of impregnating binder is maintained and the fibrous sheet is passed in contact with it so that only the side which is to be impregnated is wetted. Depth of impregnation is controlled by the temperature of the bath and time of contact of the fibrous sheet with the impregnant. With impregnating binders of the preferred type, the bath temperature is normally between about 440° F. and about 460° F. When resinous binders are used, the impregnating binder can be dispersed or dissolved in a suitable solvent and the fibrous sheet brought into contact with the dispersion to effect impregnation. The depth of impregnation is such that the impregnating binder at least contacts the sizing binder within the sheet but is less than 90 percent, and preferably less than 80 percent, of the thickness of the sheet.

The sized and impregnated fibrous sheet comprises a sized zone extending inward from one surface of the sheet and an impregnated zone extending inward from the other surface of the sheet. These zones are either contiguous within the sheet or preferably are separated by a middle or overlap zone. It is particularly undesirable for there to be dry (unimpregnated or unsized) felt within the sheet. The sized zone normally contains from about 5 to about 40 parts sizing binder and from about 0.1 to about 5 parts cured organopolysiloxane per 100 parts dry felt in the sized zone. Preferably, the sized zone contains from 15 to 35 parts sizing binder and from 0.25 to 1 part organopolysiloxane per 100 parts dry felt.

The middle or overlap zone contains sizing binder and organopolysiloxane in the same proportion based on the dry felt in the zone as are present in the sized zone. The combination of sized zone and middle zone represents from 20 to 70 percent of the thickness of the sheet with a range of 30 to 60 percent of the thickness of the sheet being particularly effective. The thickness of the combination of sized zone and middle zone is equal to the depth of penetration of the sizing solution as described hereinabove.

The impregnated zone in the case of use of a preferred bituminous impregnating binder normally contains at least 40 parts impregnating binder per 100 parts dry felt and preferably contains from 65 to 150 parts per 100 part dry felt. When resinous binders are used, the impregnated zone can contain less binder, but in any case, the proportion of binder in the impregnated zone expressed as parts binder per 100 parts dry felt in the impregnated zone must be at least 10 percent greater than the proportion of binder in the sized zone expressed as parts sizing binder per 100 parts dry felt in the sized zone. The impregnated zone represents the zone in the felt sheet which is uniformly impregnated with the impregnating binder and which contains no sizing binder or organopolysiloxane. The impregnated zone extends from the surface of the sheet opposite to that which has been sized to contact the sizing binder and organopolysiloxane within the sheet.

Although the depth of impregnation can be carefully controlled so that the impregnating binder does not penetrate into the zone which has been sized, it is preferred that a middle or overlap zone be present in the product. This middle zone can range in thickness up to about 25 percent of the sheet but is preferably from 10 percent to 20 percent of the thickness of the sheet. The presence of the organopolysiloxane tends to decrease the ease of penetration of impregnating binder into the zone, thereby causing the overlap zone to have progressively decreasing amounts of impregnating binder in the direction of the sized zone. The presence of the organopolysiloxane also inhibits the migration of impregnating binder into the sized zone during subsequent processing steps.

To the fibrous sheet containing the two or three zones as described above, there are usually applied conventional seal and backing coats. When a seal coat is used, it is applied to the surface of the impregnated zone in

such an amount that the dried coat weighs from about 0.10 to about 0.15 pound per square yard of fibrous sheet. The seal coat is commonly of either the oleoresinous or the latex types. In the case of a seal coat of the oleoresinous type, the vehicle may contain any of the drying oils or compatible resins which, after application, dry to a hard, tough consistency. For example, such drying oils as linseed oil, soy bean oil, Chinawood oil, tung oil, citicica oil and the like and such resins as rosin, ester gum, coumarone-indene resin and the like can be used. Suitable solvents such as mineral spirits, turpentine, kerosene, naphtha and the like are usually present.

In the case of a seal coat of the latex type, the vehicle comprises an aqueous emulsion of a rubber latex, such as natural rubber, butadiene-styrene copolymer, butadiene-acrylonitrile copolymer and the like. The rubber is emulsified and held dispersed by the presence of suitable dispersing agents and stabilizers.

The seal coat contains any of the conventionally used fillers, such as whiting, clay, slate flour, ground limestone, pigments and the like. Normally, the percentage of filler is between about 70 percent and about 80 percent of the weight of the dry seal coat. The seal coat is applied by such means as a flexible steel doctor blade or a roll coater.

The backing coat is formulated and applied to the surface of the sized zone in the same manner as already described in connection with the seal coat. The coat should be high in percentage of filler, in the same manner as the seal coat. The weight of the dry backing coat is normally less than about 0.25 pound per square yard of fibrous base and preferably is between 0.1 and 0.2 pound per square yard. The surface of the backing coat should be such that good adhesion with linoleum cement adhesive is provided.

After the fibrous base has been prepared comprising a sized zone or a sized zone and a middle zone, an impregnated zone, a seal coat applied to the impregnated zone and a backing coat applied to the sized zone, a layer of decorative and wear-resistant composition is applied to the side bearing the seal coat. This layer may comprise any of the well-known types used in the surface covering art. For example, a preformed sheet of linoleum composition comprising drying oil, resins and fillers can be bonded to the seal coat. Alternately, linoleum composition can be calendered directly to the felt. In this case, the seal coat is customarily omitted. Alternately, a thermoplastic resinous composition comprising such resins as polyvinyl chloride, vinyl chloride-vinyl acetate copolymer, vinylidene chloride-vinyl chloride copolymer and the like, plasticizers therefor and fillers can be bonded to the base. The decorative and wear-resistant composition can be bonded to the fibrous base without an adhesive, but an adhesive tackifier can be used if desired. The decorative layer can comprise conventional printing enamels applied by block printing, rotary or similar techniques either directly to the seal coat or to another sheet which in turn is laminated to the impregnated and sized fibrous base sheet. The printed decoration can be protected if desired by a clear wear layer comprising urea-alkyd resins, vinyl resins or the like.

When a linoleum composition is formed to a fibrous base, the product is seasoned by holding it at a temperature of between about 160° F. and 180° F. for from about two to about six weeks. When a printed decoration is applied directly to the seal coat of the fibrous base, the product is dried to remove the solvent from the printing enamels. These heating steps, in addition to insuring optimum quality in the wear layer, bring about polymerization and cross-linking to the organopolysiloxane molecule, thus producing the desirable properties in the sized zone of the fibrous base.

The fibrous base can be subjected to heat prior to application of the decorative layer to effect cure of the

organopolysiloxane. This is particularly desirable when the product receives no heat treatment after the decorative layer is applied, as in the case of a thermoplastic resinous product.

During installation, the decorative and wear-resistant product is applied to a surface to be covered by means of a suitable adhesive. Such adhesives are conventional and are preferably applied as an aqueous dispersion. The adhesive comprises a binder, such as rosin, urea-formaldehyde resin, phenol-formaldehyde resin, coumarone-indene resin, lignin, casein, synthetic or natural rubber and the like or mixtures thereof. A filler such as Portland cement, wood flour, clay and the like can also be present.

## EXAMPLE 1

Thirty-four and seven-tenths parts of asphaltic bitumen having a softening point temperature of 182° F. were dissolved in 52.1 parts of naphtha (boiling range 203° F.—290° F.).

A solution<sup>1</sup> of dimethylpolysiloxane consisting of 90 percent polymer and 10 percent xylene was prepared to meet the following specifications:

Specific gravity (77° F.) ----- 1.10  
Viscosity (77° F.) ----- centistokes 45  
Acid number \* ----- 0.1

\* Defined as the number of milligrams of potassium hydroxide required to react with 1 gram of solution.

Eighty-three hundredth parts of the polymer solution were mixed with 12.4 parts of naphtha and the resulting mixture was added to the asphalt-naphtha solution with vigorous agitation.

A sizing solution with the following composition was obtained:

|                  | Parts |
|------------------|-------|
| Asphalt          | 34.7  |
| Naphtha          | 64.5  |
| Xylene           | 0.08  |
| Siloxane polymer | 0.75  |
| 100.03           |       |

## EXAMPLE 2

One side of a felt consisting of 42 percent rag fiber, 35 percent wood pulp and 20 percent waste newsprint with a thickness of 0.045 inch was contacted with the sizing solution of Example 1 until a penetration of the solution to a depth of 0.020 inch was attained.

The felt was dried and the sized zone had the following composition:

|                  | Parts per 100<br>parts dry felt |
|------------------|---------------------------------|
| Felt             | 100                             |
| Asphalt          | 28                              |
| Siloxane polymer | 0.6                             |

The unsized side of the felt was passed in contact with a molten bath of an asphalt with a softening point of 145° F. maintained at a temperature of 450° F. The felt was impregnated a depth of 0.030 inch (.005 inch overlap zone). The impregnated zone had a composition of 100 parts of asphalt to 100 parts dry felt.

The sized and impregnated felt was coated front and back with oleoresinous seal and backing paints of conventional formulation and dried. The dry seal coat weight was 0.10 pound per square yard of felt and the backing paint weight was 0.15 pound per square yard of felt.

To the seal coat was laminated a sheet of linoleum composition consisting of 37.9 parts binder, 52.5 parts inert filler and 9.6 parts pigment. The binder consisted of 84 parts oxidized and polymerized linseed oil, 1 part lead naphthenate drier and 15 percent rosin. The filler consisted of 51 parts wood flour and 49 parts calcium car-

bonate. The product was cured by heat treatment at 170° F. for three weeks.

A covering of the linoleum type characterized by rapidity of adhesive set when bonded to a surface, freedom from tenting of seams, ability to withstand lateral shifting of the surface to which it is bonded without cracking of the wear layer, and ease of removal for replacement is produced.

## EXAMPLE 3

One side of a felt similar to that used in Example 2 was contacted with a sizing solution of the following composition:

|         | Percent by weight |
|---------|-------------------|
| Asphalt | 35                |
| Naphtha | 65                |
| 100     |                   |

The felt was dried and the sized zone had the following composition:

|         | Parts |
|---------|-------|
| Felt    | 100   |
| Asphalt | 28    |

The depth of penetration of the sizing solution into the 0.045 inch thick felt sheet was 0.020 inch.

The unsized side of the felt was passed in contact with a molten bath of asphalt maintained at a temperature of 450° F. The felt was impregnated to a depth of 0.030 inch (0.005 inch overlap zone). The impregnated zone contained 100 parts asphalt per 100 parts dry felt.

The sized and impregnated felt was coated front and back with oleoresinous seal and backing paints of conventional formulation and dried. The dry seal coat thickness was 0.10 pound per square yard of felt and the thickness of the backing paint was 0.15 pound per square yard.

A sheet of linoleum composition similar to that of Example 2 was laminated to the seal coat and the product was cured by heat treatment at 170° F. for three weeks.

A linoleum product is produced.

## EXAMPLE 4

To the backing coat of the sized and impregnated felt of Example 3 was applied a second backing coat. The felt was dried. The total dried backing coat weight was 0.32 pound per square yard of felt.

A sheet of linoleum composition similar to that of Example 2 was laminated to the seal coat and the product was cured by heat treatment at 170° F. for three weeks.

A linoleum product is produced.

Samples of the linoleums produced according to Examples 2, 3 and 4 were tested to determine the rate of adhesive setup when the product is bonded to a surface and growth when exposed to water (measure of "tenting").

The rate of adhesive setup is a qualitative test in which the adhesive is spread and the goods laid on the adhesive coated surface in the conventional manner. The linoleum is pulled up by a corner at the end of 14 hours and the degree of adhesive set estimated by observation and experience.

In the growth test, a sample of goods is laid back down loosely on a water-soaked felt pad. The growth of an 8 inch section measured across the machine direction of the felt is measured after 24 hours.

Table 1

| Exam-<br>ple No. | Siloxane<br>polymer<br>present | Backing<br>paint<br>weight<br>(lbs./sq.<br>yd.) | Percent<br>adhesive<br>set in 14<br>hours | Growth, inches per 8 inches<br>per 24 hours      |
|------------------|--------------------------------|-------------------------------------------------|-------------------------------------------|--------------------------------------------------|
| 2-----           | Yes-----                       | 0.15                                            | 90-100                                    | 0.010 in.                                        |
| 3-----           | No-----                        | 0.15                                            | 100                                       | Above 0.025 in. and extreme<br>curling tendency. |
| 4-----           | No-----                        | 0.32                                            | 20                                        | 0.018 in.                                        |

<sup>1</sup> XR-920 from Dow Corning Corporation, Midland, Michigan.

These results indicate that the presence of organosiloxane polymer in the sized zone of a sized and impregnated felt results in greatly reduced growth and tenting tendency and no loss in speed of adhesive setup as compared to felt without the polymer in the sized zone. Further, when compared with felt with two backing coats, which the prior art has found necessary, the felt with siloxane polymer in the sized zone exhibits much more rapid adhesive setup and even some improvement in rate of growth.

## EXAMPLE 5

Twenty-four parts of asphalt having a softening point temperature of 175° F. are dissolved in 74 parts of toluene and to this solution is added 2 parts of a 50 percent solution of methyl hydrogen polysiloxane<sup>2</sup> in xylene.

A sizing solution with the following composition was obtained:

|                  | Parts |
|------------------|-------|
| Asphalt          | 24    |
| Toluene          | 74    |
| Xylene           | 1     |
| Siloxane polymer | 1     |
|                  | 100   |

One side of a 0.043 inch thick all rag felt (50 percent mattresses, 25 percent rags and 25 percent cotton cuttings) was sized with the sizing solution to a depth of penetration of 0.024. The felt was dried and the sized zone had the following composition:

|                  | Parts per 100 parts dry felt |
|------------------|------------------------------|
| Felt             | 100                          |
| Asphalt          | 21                           |
| Siloxane polymer | 0.9                          |

The unsized side of the felt was contacted with a molten bath of asphalt maintained at a temperature of 465° F. The felt was impregnated to a depth of .025 inch (0.006 inch overlap zone). The impregnated zone had a composition of 105 parts asphalt to 100 parts dry felt.

The sized and impregnated felt was coated front and back with oleoresinous seal and backing paints of conventional formulation and dried. The dry seal coat weight on the impregnated side of the felt and the backing paint weight on the sized side of the felt was 0.13 pound per square yard.

The product is suitable as a backing material for a surface covering product.

## EXAMPLE 6

To the seal coat of the product of Example 5 was laminated a sheet of linoleum composition with a composition consisting of 37.9 parts binder, 52.5 parts inert filler and 9.6 parts pigment. The binder consisted of 84 percent oxidized and polymerized linseed oil, 1 percent lead naphthenate drier and 15 percent rosin. The filler consisted of 51 percent wood flour and 49 percent calcium carbonate.

The uncured linoleum on the felt backing was cured at 170° F. for 26 days. A linoleum product characterized by rapid adhesion to a surface and freedom from tenting tendencies is produced.

## EXAMPLE 7

The product of Example 2 was fed to a conventional block printing machine and on the seal coat was printed a decorative pattern with standard printing enamels. A typical printing enamel composition is formulated by mixing 100 parts pigments and extenders and 42 parts vehicle consisting of 50 percent linseed and soy bean oils, 27 percent phenolic and alkyd resins, 14 percent naphtha and 1 percent metallic driers to form a thick smooth

paste. This paste is thinned with additional vehicle to produce an enamel of the proper consistency.

The printed sheet leaving the block printing machine is dried for 3 days at 155° F. The decorative product is characterized by ease of adhesion to a surface and freedom from tenting tendencies of the seams.

## EXAMPLE 8

The following mixture is heated for 3 minutes in a Banbury mixer at 300° F.:

|                                        | Parts by weight |
|----------------------------------------|-----------------|
| Vinyl chloride-vinyl acetate copolymer | 243             |
| Tricresyl phosphate                    | 131             |
| Asbestos                               | 155             |
| 15 Wood flour                          | 40              |
| Silica flour                           | 325             |
| Stearic acid                           | 1               |
| Basic lead carbonate                   | 5               |
| Titanium dioxide                       | 100             |

The mixture is sheeted between hot metal rolls at 325° F. to produce a smooth sheet of resin composition.

To the seal coat of the product of Example 2 is applied a coating of an adhesive composition comprising 65 parts 25 butadiene-acrylonitrile copolymer latex of 50 percent solids and 35 parts "Vinsol." "Vinsol," made by Hercules Powder Company, is a hard, dark, thermoplastic resin with a melting point between 234° F. and 239° F. which is a byproduct in the extraction of wood rosin from pine stumps.

The coated felt is dried and then the adhesive coating is activated by heating to about 235° F. The smooth resin composition sheet is laminated to the adhesive coated felt to produce a product characterized by ease of adhesion to a surface and freedom from severe tenting tendencies.

Although the fibrous sheet produced in accordance with the invention has been described as being useful as a backing for a surface covering product, it may be used alone 40 as a lining felt which is interposed between a flexible smooth surface covering and a subfloor and which is bonded both to the overlying covering and to the subfloor by suitable adhesives. When the fibrous sheet is used as a lining felt, it ordinarily is used without either seal or backing coats.

Any departure from the above description which conforms to the present invention is intended to be included within the scope of the claims.

I claim:

1. In a method of treating a felted fibrous sheet to render it suitable as a backing for a smooth surface covering for floors, walls and the like which comprises impregnating from one surface of the sheet to a depth of about 20 to about 70 percent of the thickness of the sheet with a dispersion in a volatile solvent of a sizing binder selected from the group consisting of bituminous binders and organic resinous binders thereby forming a first zone in said sheet and thereafter impregnating from the opposite surface of the sheet to a depth sufficient to at least contact the first zone but less than 90 percent of the thickness of the sheet with an impregnating binder selected from the group consisting of bituminous binders and organic resinous binders thereby forming a second zone in said sheet, there being at least 10 percent greater percentage of binder in said second zone than in said first zone, the improvement which comprises uniformly incorporating in said dispersion of sizing binder a heat-hardenable organopolysiloxane having a molecular structure comprising repeating units of the radical



wherein R<sub>1</sub> is a hydrocarbon group containing from 1 to 8 carbon atoms and R<sub>2</sub> is selected from the group con-

sisting of hydrocarbon groups containing from 1 to 8 carbon atoms and hydrogen, thereby incorporating in said first zone from about 0.1 to about 5 percent of said organopolysiloxane based on the weight of the dry sheet in the first zone.

2. The method according to claim 1 wherein said organopolysiloxane has a viscosity of about 5 to about 5,000 centistokes when measured at 77° F. in a mixture of 90 percent of the organopolysiloxane and 10 percent xylene.

3. In a method of treating a felted fibrous sheet to render it suitable as a backing for a smooth surface covering for floors, walls and the like which comprises impregnating from one surface of the sheet to a depth of about 20 to about 70 percent of the thickness of the sheet with a dispersion in a volatile solvent of a bituminous sizing binder thereby forming a first zone in said sheet and thereafter impregnating from the opposite surface of the sheet to a depth sufficient to at least contact the first zone but less than 90 percent of the thickness of the sheet with a bituminous impregnating binder thereby forming a second zone in said sheet, there being at least 10 percent greater percentage of binder in said second zone than in said first zone, the improvement which comprises uniformly incorporating in said dispersion of sizing binder a heat-hardenable organopolysiloxane having a molecular structure comprising repeating units of the radical



wherein R<sub>1</sub> is a hydrocarbon group containing from 1 to 8 carbon atoms and R<sub>2</sub> is selected from the group consisting of hydrocarbon groups containing from 1 to 8 carbon atoms and hydrogen, thereby incorporating in said first zone from about 0.1 to about 5 percent of said organopolysiloxane based on the weight of the dry sheet in the first zone.

4. The method according to claim 3 wherein said organopolysiloxane has a viscosity of about 5 to about 5,000 centistokes when measured at 77° F. in a mixture of 90 percent of the organopolysiloxane and 10 percent xylene.

5. A fibrous sheet comprising an impregnated zone, a middle zone and a sized zone, said impregnated zone extending inward from one surface of said sheet and said sized zone extending inward from the opposite surface of said sheet, said impregnated zone and said sized zone being separated within said sheet by said middle zone, said sized zone and said middle zone constituting about 20 to about 70 percent of the thickness of the sheet and being uniformly sized with about 5 to about 40 percent of a bituminous sizing binder by weight and 0.25 to 1 percent of a cured organopolysiloxane by weight, the weights being based on the weight of dry sheet in said sized zone and said middle zone, said bituminous sizing binder having a softening point between about 130° F. and about 200° F., said organopolysiloxane having a molecular structure comprising repeating units of the radical



wherein R<sub>1</sub> is a hydrocarbon group containing from 1 to 8 carbon atoms and R<sub>2</sub> is selected from the group consisting of hydrocarbon groups containing from 1 to 8 carbon atoms and hydrogen and having a viscosity of about 5 to about 5,000 centistokes when measured at 77° F. in a mixture of 90 percent of the organopolysiloxane and 10 percent xylene, the impregnated zone being

uniformly impregnated with more than 40 percent of a bituminous impregnating binder by weight based on the weight of the dry sheet in the impregnated zone, the ratio of the impregnating binder to the dry sheet in the impregnated zone being at least 10 percent greater than

5 the ratio of the sizing binder to the dry sheet in the sized zone and the middle zone, said bituminous impregnating binder having a softening point between about 100° F. and about 160° F. and said middle zone having 10 a thickness of less than 25 percent of the thickness of said sheet and comprising the bituminous impregnating binder in an amount progressively decreasing within said middle zone from the impregnated zone towards the sized zone.

15 6. In a method of treating a felted fibrous sheet to render it suitable as a backing for a smooth surface covering for floors, walls and the like which comprises impregnating from one surface of the sheet to a depth of about 20 to about 70 percent of the thickness of the sheet with a dispersion in a volatile solvent of a bituminous sizing binder having a softening point of about 130° F. to about 200° F. thereby forming a first zone in said sheet and thereafter impregnating from the opposite surface of the sheet to a depth sufficient to at least

20 contact the first zone but less than 90 percent of the thickness of the sheet with a bituminous impregnating binder having a softening point of about 100° F. to about 160° F. thereby forming a second zone in said sheet, said first zone comprising about 5 to about 40

25 percent of the bituminous sizing binder by weight based on the weight of the dry sheet in said first zone and said second zone comprising at least 40 percent of the bituminous impregnating binder by weight based on the weight of the dry sheet in said second zone, the ratio of the impregnating binder to the dry sheet in said second zone being at least 10 percent greater than the ratio

30 of the sizing binder to the dry sheet in said first zone, the improvement which comprises uniformly incorporating in said dispersion of sizing binder a heat-hardenable organopolysiloxane having a molecular structure comprising repeating units of the radical

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9

percent of the bituminous sizing binder by weight based on the weight of the dry sheet in said first zone and said second zone comprising from 65 percent to 150 percent of the bituminous impregnating binder by weight based on the weight of the dry sheet in said second zone, the improvement which comprises uniformly incorporating in said dispersion of sizing binder about 0.2 to about 10 percent by weight of a heat-hardenable organopolysiloxane having a molecular structure comprising repeating units of the radical



wherein  $R_1$  is a hydrocarbon group containing from 1 to 8 carbon atoms and  $R_2$  is selected from the group consisting of hydrocarbon groups containing from 1 to 8 carbon atoms and hydrogen, said organopolysiloxane having a viscosity of about 5 to about 5,000 centistokes when measured at 77° F. in a mixture of 90 percent of the organopolysiloxane and 10 percent xylene, thereby incorporating in said first zone from about 0.1 to about 5 percent of said organopolysiloxane based on the weight of the dry sheet in the first zone.

9. The method according to claim 8 wherein said organopolysiloxane has a viscosity of 10 to 100 centistokes when measured at 77° F. in a mixture of 90 percent of organopolysiloxane and 10 percent xylene.

10. The method according to claim 9 wherein said dispersion contains 0.5 to 1.25 percent of said organopolysiloxane by weight and wherein said first zone contains from 0.25 to 1 percent of said organopolysiloxane by weight based on the weight of the dry sheet in the first zone.

11. The method according to claim 10 wherein said organopolysiloxane is methyl hydrogen polysiloxane.

12. The method according to claim 10 wherein said organopolysiloxane is dimethylpolysiloxane.

13. In a method of treating a felted fibrous sheet to render it suitable as a backing for a smooth surface covering for floors, walls and the like which comprises impregnating from one surface of the sheet to a depth of about 20 to about 70 percent of the thickness of the sheet with a dispersion in a volatile solvent comprising about 10 to about 50 percent by weight of a bituminous sizing binder having a softening point of 170° F. to 190° F. thereby forming a first zone in said sheet, drying said sheet to remove said solvent and thereafter impregnating from the opposite surface of the sheet to a depth sufficient to at least contact the first zone but less than 90 percent of the thickness of the sheet with a bituminous impregnating binder having a softening point of 140° F. to 150° F. thereby forming a second zone in said sheet, said first zone comprising about 5 to about 40 percent of the bituminous sizing binder by weight based on the weight of the dry sheet in said first zone and said second zone comprising from 65 percent to 150 percent of the bituminous impregnating binder by weight based on the weight of the dry sheet in said second zone, the improvement which comprises uniformly incorporating in said dispersion of sizing binder a heat-hardenable organopolysiloxane having a molecular structure comprising repeating units of the radical



wherein  $R_1$  is a hydrocarbon group containing from 1 to 8 carbon atoms and  $R_2$  is selected from the group consisting of hydrocarbon groups containing from 1 to 8 carbon atoms and hydrogen, thereby incorporating in said first zone from about 0.1 to about 5 percent of said

organopolysiloxane based on the weight of the dry sheet in the first zone.

14. The method according to claim 13 wherein said organopolysiloxane has a viscosity of about 5 to about 5,000 centistokes when measured at 77° F. in a mixture of 90 percent of the organopolysiloxane and 10 percent xylene.

15. The method according to claim 14 wherein said organopolysiloxane is methyl hydrogen polysiloxane.

16. The method according to claim 14 wherein said organopolysiloxane is dimethylpolysiloxane.

17. In a flexible felted fibrous sheet comprising a first zone and a second zone, said first zone extending from one surface of the sheet to a substantial depth and being uniformly sized with about 5 to about 40 percent by weight based on the weight of the dry sheet in said first zone of a sizing binder selected from the group consisting of bituminous binders and organic resinous binders and said second zone extending from the opposite surface of the sheet to contact said first zone and being uniformly impregnated with an impregnating binder selected from the group consisting of bituminous binders and organic resinous binders, the ratio of the impregnating binder to the dry sheet in said second zone being at least 10 percent greater than the ratio of the sizing binder to the dry sheet in said first zone, the improvement which comprises incorporating uniformly in said first zone about 0.1 to about 5 percent of a cured organopolysiloxane based on the weight of the dry sheet in said first zone, said organopolysiloxane having molecular structure comprising repeating units of the radical



wherein  $R_1$  is a hydrocarbon group containing from 1 to 8 carbon atoms and  $R_2$  is selected from the group consisting of hydrocarbon groups containing from 1 to 8 carbon atoms and hydrogen.

18. In a flexible felted fibrous sheet comprising a first zone and a second zone, said first zone extending from one surface of the sheet to a depth of between 20 percent and 70 percent of the thickness of the sheet and being uniformly sized with about 5 to about 40 percent of a bituminous sizing binder by weight based on the weight of the dry sheet in said first zone, said bituminous sizing binder having a softening point of about 130° F. to about 200° F. and said second zone extending from the opposite surface of said sheet to at least contact said first zone and being uniformly impregnated with a bituminous impregnating binder having a softening point of about 100° F. to about 160° F., the ratio of the impregnating binder to the dry sheet in said second zone being at least 10 percent greater than the ratio of the sizing binder to the dry sheet in said first zone, the improvement which comprises incorporating uniformly in said first zone about 0.1 to about 5 percent of a cured organopolysiloxane, said organopolysiloxane having a molecular structure comprising repeating units of the radical.



wherein  $R_1$  is a hydrocarbon group containing from 1 to 8 carbon atoms and  $R_2$  is selected from the group consisting of hydrocarbon groups containing from 1 to 8 carbon atoms and hydrogen, said organopolysiloxane having a viscosity of about 5 to 5,000 centistokes when measured at 77° F. in a mixture of 90 percent organopolysiloxane and 10 percent xylene.

19. The flexible felted fibrous sheet according to claim 18 wherein said organopolysiloxane has a viscosity of 10 to 100 centistokes when measured at 77° F. in a mix-

## 15

ture of 90 percent organopolysiloxane and 10 percent xylene.

20. The flexible felted fibrous sheet of claim 19 wherein said first zone contains 0.25 to 1 percent cured organopolysiloxane.

21. In a flexible felted fibrous sheet comprising a first zone and a second zone, said first zone extending from one surface of the sheet to a depth of between 20 percent and 70 percent of the thickness of the sheet and being uniformly sized with 15 to 35 percent of a bituminous sizing binder by weight based on the weight of the dry sheet in said first zone, said bituminous sizing binder having a softening point of about 130° F. to about 200° F. and said second zone extending from the opposite surface of the sheet to at least contact said first zone and being uniformly impregnated with 65 percent to 150 percent of a bituminous impregnating binder by weight based on the weight of the dry sheet in said second zone, said bituminous impregnating binder having a softening point of about 100° F. to about 160° F., the improvement which comprises incorporating uniformly in said first zone 0.25 to 1.25 percent of a cured organopolysiloxane, said organopolysiloxane having a molecular structure comprising repeating units of the radical



wherein R<sub>1</sub> is a hydrocarbon group containing from 1 to 8 carbon atoms and R<sub>2</sub> is selected from the group consisting of hydrocarbon groups containing from 1 to 8 carbon atoms and hydrogen, said organopolysiloxane having a viscosity of about 5 to 5,000 centistokes when measured at 77° F. in a mixture of 90 percent organopolysiloxane and 10 percent xylene.

22. The flexible felted fibrous sheet according to claim 21 wherein said organopolysiloxane is methyl hydrogen polysiloxane.

23. The flexible felted fibrous sheet according to claim 21 wherein said organopolysiloxane is dimethylpolysiloxane.

24. In a resilient smooth surface covering for floors, walls and the like, which comprises a flexible felted fibrous backing sheet comprising a first zone and a second zone, said first zone extending from one surface of the sheet to a depth of between 20 percent and 70 percent of the thickness of the sheet and being uniformly sized with about 5 per cent to about 40 percent of a bituminous sizing binder by weight based on the weight of the dry sheet in said first zone, said bituminous sizing binder having a softening point of about 130° F. to about 200° F. and said second zone extending from the opposite surface of said sheet to at least contact said first zone and being uniformly impregnated with a bituminous impregnating binder having a softening point of about 100° F. to about 160° F., the ratio of the bituminous impregnating binder to the dry sheet in said second zone being at least 10 percent greater than the ratio of the sizing binder to the dry sheet in said first zone, and bonded to said opposite surface bearing said second zone a layer of decorative and wear-resistant composition, the improvement which comprises incorporating uniformly in said first zone about 0.1 to about 5 percent of a cured organopolysiloxane, said organopolysiloxane having a molecular structure comprising repeating units of the radical



wherein R<sub>1</sub> is a hydrocarbon group containing from 1 to 8 carbon atoms and R<sub>2</sub> is selected from the group consisting of hydrocarbon groups containing from 1 to 8 carbon

## 16

atoms and hydrogen, said organopolysiloxane having a viscosity of about 5 to 5,000 centistokes when measured at 77° F. in a mixture of 90 percent organopolysiloxane and 10 percent xylene.

5. 25. The fibrous sheet according to claim 5 wherein said middle zone has a thickness of between 10 percent and 20 percent of the thickness of said sheet.

10. 26. In a method of treating a felted fibrous sheet to render it suitable as a backing for smooth surface coverings for floors, walls and the like which comprises impregnating from one surface of the sheet to a depth of 30 to 60 percent of the thickness of the sheet with a dispersion in a volatile solvent of a bituminous sizing binder having a softening point of about 130° F. to about 200° F. thereby forming a first zone in said sheet and thereafter impregnating from the opposite surface of the sheet to a depth sufficient to at least contact the first zone but less than 80 percent of the thickness of the sheet with a bituminous impregnating binder having a softening point of about 100° F. to about 160° F. thereby forming a second zone in said sheet, said first zone comprising about 5 percent to about 40 percent of the bituminous sizing binder by weight based on the weight of the dry sheet in said first zone and said second zone comprising at least 40 percent of the bituminous impregnating binder by weight based on the weight of the dry sheet in said second zone, the ratio of the impregnating binder to the dry sheet in said second zone being at least 10 percent greater than the ratio of the sizing binder to the dry sheet in said first zone, the improvement which comprises uniformly incorporating in said dispersion of sizing binder a heat-hardenable organopolysiloxane having a molecular structure comprising repeating units of the radical



30. 35. wherein R<sub>1</sub> is a hydrocarbon group containing from 1 to 8 carbon atoms and R<sub>2</sub> is selected from the group consisting of hydrocarbon groups containing from 1 to 8 carbon atoms and hydrogen, said organopolysiloxane having a viscosity of about 5 to about 5,000 centistokes when measured at 77° F. in a mixture of 90 percent of the organopolysiloxane and 10 percent xylene.

40. 45. 27. The method according to claim 26 wherein said bituminous sizing binder has a softening point of 170 to 190° F. and said bituminous impregnating binder has a softening point of 140 to 150° F.

50. 28. The method according to claim 26 wherein said dispersion contains 20 to 40 percent of said bituminous sizing binder by weight.

55. 29. The method according to claim 26 wherein said impregnating binder penetrates into said first zone for a distance of less than about 25 percent of the thickness of said sheet.

60. 30. The method according to claim 26 wherein said impregnating binder penetrates into said first zone for a distance of between 10 percent and 20 percent of the thickness of said sheet.

31. The method according to claim 29 wherein said organopolysiloxane is methyl hydrogen polysiloxane.

32. The method according to claim 29 wherein said organopolysiloxane is dimethylpolysiloxane.

65. 33. In a flexible felted fibrous sheet comprising a first zone and a second zone, said first zone extending from one surface of the sheet to a depth of between 20 percent and 70 percent of the thickness of the sheet and being uniformly sized with about 5 to about 40 percent of a bituminous sizing binder by weight based on the weight of the dry sheet in said first zone and said second zone extending from the opposite surface of said sheet to at least contact said first zone and being uniformly impregnated with a bituminous impregnating binder, the ratio of the impregnating binder to the dry sheet in said second zone being at least 10 percent greater than the ratio of the

17

sizing binder to the dry sheet in said first zone, the improvement which comprises incorporating uniformly in said first zone about 0.1 to about 5 percent of a cured organopolysiloxane, said organopolysiloxane having a molecular structure comprising repeating units of the radical



10

wherein  $\text{R}_1$  is a hydrocarbon group containing from 1 to 8

18

carbon atoms and  $\text{R}_2$  is selected from the group consisting of hydrocarbon groups containing from 1 to 8 carbon atoms and hydrogen, said organopolysiloxane having a viscosity of about 5 to 5,000 centistokes when measured at 77° F. in a mixture of 90 percent organopolysiloxane and 10 percent xylene.

## References Cited in the file of this patent

## UNITED STATES PATENTS

|           |             |               |
|-----------|-------------|---------------|
| 2,295,070 | Allen ----- | Sept. 8, 1942 |
| 2,527,793 | Bump -----  | Oct. 31, 1950 |

UNITED STATES PATENT OFFICE  
CERTIFICATE OF CORRECTION

Patent No. 2,849,335

Leon B. Palmer

August 26, 1958

It is hereby certified that error appears in the above numbered patent requiring correction and that the said Letters Patent should read as corrected below.

In the heading of the printed specification, between lines 7 and 8, insert the following:

— Continuation-in-part of S. N. 427,229 filed May 3, 1954 —; column 7, line 59, after "impregnated" insert — to —; column 9, line 7, for "felt was" read — felt with —; line 29, for "penetration" read — penetration —; column 10, line 10, for "300° F." read — 330° F. —.

Signed and sealed this 16th day of June 1959.

(SEAL)  
Attest:

KARL H. AXLINE  
Attesting Officer

ROBERT C. WATSON  
Commissioner of Patents